

## UNITED STATES PATENT OFFICE

2,428,959

## ZINC-TITANIUM-MANGANESE ALLOYS

Edward J. Boyle and Edmund A. Anderson,  
Palmerton, Pa., assignors to The New Jersey  
Zinc Company, New York, N. Y., a corporation  
of New Jersey

No Drawing. Application May 17, 1944,  
Serial No. 536,016

10 Claims. (Cl. 75—178)

**1** This invention relates to zinc base alloys and more particularly to zinc base alloys containing titanium, and aims to provide an improved zinc base alloy containing titanium and manganese. By "zinc base" alloy is meant an alloy containing at least about 97% zinc.

The zinc base alloys of the invention contain from 0.01 to 1.6%, and preferably from 0.05 to 0.5%, titanium and are characterized by additionally containing from 0.05 to 1.5%, and preferably from 0.1 to 1%, of manganese. The balance of the alloy is substantially all zinc. Alloys of the invention may advantageously contain about 0.1% titanium, 0.3 to 0.6% manganese, and the balance zinc. The zinc base of the alloys is preferably high grade zinc. Alloys of superior creep resistance, that is resistance to prolonged static loads well below the ultimate limit, and of fine grain size when cast result from the use, as the zinc base, of metal of high purity, such as zinc at least 99.99% pure. On the other hand, satisfactory alloys are obtained with zinc of the grade commonly used in the production of commercial rolled zinc, for example zinc metal containing 0.10% lead, 0.012% iron and 0.005% cadmium. The presence of 0.1% lead is sufficient, however, to impart to the alloys (as cast) a coarse, columnar grain structure similar to that of ordinary cast zinc. If the alloy is rolled or otherwise mechanically worked, the coarse grain structure of the cast alloy disappears, and the micro-structure and properties of the rolled or worked alloy are substantially independent of the grade or purity of the zinc base within the limits hereinbefore mentioned.

The alloys of the invention are particularly adapted for rolling. When transformed to sheet or strip by suitable rolling procedure, the alloys possess high creep resistance. The alloys may be hot rolled at metal temperatures of from 150 to 300° C., temperatures of from 200 to 240° C. giving very satisfactory results. The hot rolling may be a finishing operation consisting of say three or more passes through the rolls, and may be applied to metal either hot or cold rolled prior to the hot finishing. Cold rolling tends to decrease the creep resistance, but the characteristic high creep resistance can be substantially restored by subsequent heat treatment such, for example, as annealing for a short period at a temperature of from 150 to 400° C., annealing in oil for about five minutes at a temperature of about 275° C. giving very satisfactory results. Cold rolling, at least in the final stages, imparts to the alloy certain advantages, especially with respect to tensile

elongation. Alloys of the invention are to be considered cold rolled when the rolling (or other mechanical working) is carried out under thermal conditions resulting in a temperature of the rolled strip or sheet after the final rolling pass (final coil temperature) due simply to the mechanical working, and are to be considered hot rolled when the rolling is carried out under thermal conditions resulting in a final coil temperature of from 10 150 to 300° C., and preferably from 200 to 240° C.

In the production of the alloys of the invention, it is preferable to prepare an intermediate zinc base alloy containing a relatively high proportion of titanium. Conveniently, the intermediate alloy may contain about 4% of titanium, and is prepared by heating a mixture of 96 parts of zinc and 4 parts of titanium in a clay-carborundum crucible at a temperature of 800° C. for about 8 hours. The intermediate alloy is cast 15 into a thin slab and crushed to a convenient size for alloying. The final titanium content of the cast intermediate alloy usually does not depart far from the contemplated 4%. Manganese is preferably introduced into the alloy by preparing 20 an intermediate zinc alloy of high manganese content. The intermediate alloys, in calculated amounts to give the desired titanium and manganese contents, are mixed with zinc metal and melted together and held at a temperature of 25 about 500° C. for an hour or so. Very little titanium or manganese is lost in this heating.

The alloys of the invention are characterized by high creep resistance, dynamic ductility, tensile strength, tensile elongation and good bending 30 properties. These characteristics, among others, of the alloys are shown in the following table. In the table, "H" is sclerometer hardness; "D. D." is dynamic ductility and is measured as the maximum depth in inches of a cup that can be formed 35 by a standard plunger in an uncut sheet of the metal without fracture; "Tem." is percent temper, and is determined by the degree to which a standard test strip returns to its original position after being wrapped around a mandrel; 40 "T. S." is tensile strength (with the grain) in pounds per square inch; "T. E." is tensile elongation (with the grain), in percent in a 2 inch test strip; and "C. R." is the creep rate or creep resistance (with the grain) expressed as the inverse creep rate (the more creep resistant alloy having the higher inverse creep rate) which is the number of units of time (days) required to produce an elongation or creep (with the grain) of one percent (i. e. days per %) in a standard test 45 piece when subjected to dead loads of 8,000 and 50

12,000 pounds (respectively) per square inch at constant room temperature (25° C.). The cold bend values represent the diameter of uncracked 180° bends in multiples of sheet thickness (gauge), and the lower values indicate better bending properties. "Cut and draw" is the result of an actual drawing operation carried out on a disc cut from the sheet, and the figures given represent the percent decrease in diameter of the cup, as compared with the blank (percent take-in). The columns headed by the single asterisk (\*) and by the double asterisk (\*\*) are results obtained with test pieces as rolled and as annealed for five minutes at 275° C. in oil, respectively. The titanium (Ti) and manganese (Mn) contents of the alloys given in the table are the amounts of these alloying metals added to the zinc base which was high purity metal. The alloys were compounded in the manner hereinbefore described.

from 0.01 to 1.6% titanium and from 0.05 to 1.5% manganese and the balance essentially all zinc.

5 6. A hot rolled zinc base alloy containing at least about 97% zinc and characterized by high creep resistance and containing from 0.01 to 1.6% titanium and from 0.05 to 1.5% manganese and the balance essentially all zinc.

10 7. A cold rolled and annealed zinc base alloy containing at least about 97% zinc and characterized by high creep resistance and containing from 0.05 to 0.5% titanium and from 0.1 to 1% manganese and the balance essentially all zinc.

15 8. A zinc base alloy according to claim 7 containing about 0.1% titanium and from 0.3 to 0.6% manganese.

20 9. A hot rolled zinc base alloy containing at least about 97% zinc and characterized by high creep resistance and containing from 0.05 to 0.5% titanium and from 0.1 to 1% manganese and the

Table

| Ti                                                                                                                                                                              | Mn  | Test Gauge | H    | D. D. | Tem. | Cold Bends |              | T. S. | T. E. | Creep Resistance |    |   |        | Cut and draw |      |      |       |         |       |       |      |
|---------------------------------------------------------------------------------------------------------------------------------------------------------------------------------|-----|------------|------|-------|------|------------|--------------|-------|-------|------------------|----|---|--------|--------------|------|------|-------|---------|-------|-------|------|
|                                                                                                                                                                                 |     |            |      |       |      | With Grain | Across Grain |       |       | *                | ** | * | **     | *            | **   |      |       |         |       |       |      |
| .1                                                                                                                                                                              | .05 | .0145      | 22   | 20    | .290 | .300       | 47           | 43    | 3     | 2½               | 2  | 2 | 22,800 | 22,500       | 33.7 | 23.8 | 1.53  | 434.8   | .040  | 33.8  | 40.8 |
| .1                                                                                                                                                                              | .10 | .0185      | 23   | 20    | .305 | .305       | 46           | 42    | 3     | 3                | 2  | 2 | 23,600 | 23,100       | 39.5 | 30.3 | 1.39  | 400.0   | .045  | 79.4  | 41.2 |
| .1                                                                                                                                                                              | .20 | .018       | 24   | 20    | .315 | .305       | 45           | 44    | 3     | 3                | 2  | 2 | 24,900 | 22,900       | 41.0 | 35.8 | 1.61  | 555.6   | .066  | 131.6 | 41.4 |
| .1                                                                                                                                                                              | .30 | .018       | 24   | 22    | .315 | .305       | 46           | 46    | 3     | 3                | 2  | 2 | 24,400 | 24,100       | 45.2 | 33.2 | 4.46  | 476.2   | .084  | 243.9 | 42.1 |
| .1                                                                                                                                                                              | .40 | .017       | 26   | 24    | .310 | .300       | 46           | 48    | 3     | 3                | 2  | 2 | 25,000 | 23,700       | 39.9 | 30.5 | 4.06  | 1,000.0 | .013  | 256.4 | 41.5 |
| Rolling Treatment: Slab heated to 275° C., rough rolled to 0.09" in six passes; cold coil rolled on hot rolls to 0.018" in four passes, final coil temperature about 160° C.    |     |            |      |       |      |            |              |       |       |                  |    |   |        |              |      |      |       |         |       |       |      |
| .1                                                                                                                                                                              | .05 | .0155      | 25   | 16.5  | .285 | .310       | 47           | 40    | 5     | 4½               | 2  | 2 | 22,500 | 19,300       | 56.0 | 28.5 | .097  | 500.0   | .0039 | 2.11  | 40.8 |
| .1                                                                                                                                                                              | .10 | .0165      | 27   | 18    | .320 | .300       | 46           | 42    | 5     | 2½               | 2  | 2 | 23,000 | 20,700       | 66.8 | 34.3 | .12   | 384.6   | .007  | 22.4  | 40.9 |
| .1                                                                                                                                                                              | .20 | .0175      | 28   | 22    | .320 | .300       | 44           | 44    | 5     | 3                | 2  | 2 | 23,600 | 23,500       | 75.2 | 27.2 | .33   | 526.3   | .011  | 232.6 | 40.9 |
| .1                                                                                                                                                                              | .30 | .0175      | 29   | 25    | .330 | .295       | 44           | 48    | 5     | 3½               | 2  | 2 | 24,100 | 25,600       | 70.2 | 23.0 | .78   | 79.2    | .018  | 500.0 | 41.1 |
| .1                                                                                                                                                                              | .40 | .018       | 29.5 | 26    | .330 | .290       | 42           | 48    | 4½    | 4                | 2  | 2 | 23,000 | 27,000       | 68.3 | 29.0 | .70   | 526.3   | .020  | 370.4 | 41.3 |
| Rolling Treatment: Slab heated to 275° C., rough rolled to 0.09" in six passes; cold coil rolled on hot rolls to 0.036" in three passes; cold rolled to 0.018" in three passes  |     |            |      |       |      |            |              |       |       |                  |    |   |        |              |      |      |       |         |       |       |      |
| .1                                                                                                                                                                              | .50 | .018       | 28   | 26    | .305 | .270       | 41           | 48    | 3½    | 4½               | 2  | 2 | 20,700 | 26,600       | 78.8 | 25.8 | .87   | 476.2   | .011  | 243.9 | 38.3 |
| Rolling Treatment: Slab heated to 230-280° C., rough rolled to 0.09" in ten passes; cold coil rolled on warm rolls to 0.018" in five passes, final coil temperature 90-130° C.  |     |            |      |       |      |            |              |       |       |                  |    |   |        |              |      |      |       |         |       |       |      |
| .1                                                                                                                                                                              | .5  | .0135      | 27.5 | 26    | .270 | .270       | 49           | 52    | 3     | 4                | 2  | 2 | 22,500 | 26,800       | 37.8 | 26.5 | 128.2 | 666.7   | .69   | 250.0 | 40.8 |
| Rolling Treatment: Slab heated to 230-280° C., rough rolled to 0.09" in ten passes; cold coil rolled on hot rolls to 0.018" in three passes, final coil temperature 160-185° C. |     |            |      |       |      |            |              |       |       |                  |    |   |        |              |      |      |       |         |       |       |      |

\*As rolled. \*\*As annealed.

We claim:

1. A zinc base alloy containing at least about 55 97% zinc and characterized by high creep resistance containing from 0.01 to 1.6% titanium and from 0.05 to 1.5% manganese and the balance zinc.

2. A zinc base alloy containing at least about 60 97% zinc and characterized by high creep resistance containing from 0.05 to 0.5% titanium and from 0.1 to 1% manganese and the balance zinc.

3. A zinc base alloy containing at least about 65 97% zinc and characterized by high creep resistance containing about 0.1% titanium and from 0.3 to 0.6% manganese and the balance zinc.

4. A zinc base alloy containing at least about 70 97% zinc and characterized by high creep resistance containing about 0.1% titanium and about 0.5% manganese and the balance zinc.

5. A cold rolled and annealed zinc base alloy containing at least about 97% zinc and characterized by high creep resistance and containing

balance essentially all zinc.

10. A zinc base alloy according to claim 9 containing about 0.1% titanium and from 0.3 to 0.6% manganese.

EDWARD J. BOYLE.  
EDMUND A. ANDERSON.

#### REFERENCES CITED

The following references are of record in the file of this patent:

#### UNITED STATES PATENTS

| Number    | Name   | Date          |
|-----------|--------|---------------|
| 1,020,512 | Rossi  | Mar. 19, 1912 |
| 1,335,284 | Hodson | Mar. 30, 1920 |
| 2,048,288 | Pierce | July 2, 1936  |
| 2,317,179 | Daesen | Apr. 20, 1943 |

#### OTHER REFERENCES

Metals Handbook, 1939 edition, pages 1737, 1765, published by American Society for Metals, Cleveland, Ohio.